

Patented Mar. 19, 1935

**1,994,563**

UNITED STATES PATENT OFFICE

1,994,563

# THIAZOLOCARBOCYANINE DYE AND PROCESS OF PREPARING IT

**Leslie G. S. Brooker, Rochester, N. Y., assignor to  
Eastman Kodak Company, Rochester, N. Y., a  
corporation of New York**

No Drawing. Application June 29, 1932,  
Serial No. 619,962

**16 Claims. (Cl. 260—44)**

This invention relates to new compounds and particularly to a new class of photographic sensitizing dyes, termed thiazolocarbocyanines, and methods for the preparation thereof.

5 In my co-pending application No. 548,025, it  
was mentioned that certain dyes, for which the  
name "neothiazolocarbocyanine" is proposed,  
could be prepared from bases of the thiazole se-  
ries. It was further stated in that application  
10 that these neothiazolocarbocyanines were pro-  
duced when certain alkyl quaternary salts of the  
thiazoles were treated with ethyl orthoformate  
in pyridine solution. The alkyl quaternary salts  
of the bases which are most suitable for the prep-  
15 aration of the neothiazolocarbocyanines are those  
of alkylsulfuric acids or, better still, arylsulfonic  
acids. It was further mentioned in my above  
application that in general a proportion of nor-  
20 mal thiazolocarbocyanine accompanied the neo-  
thiazolocarbocyanine, and in most instances the  
normal thiazolocarbocyanine was more soluble  
than the neothiazolocarbocyanine and the latter  
could therefore be readily obtained in a state of  
purity.

25 It was stated in addition that the normal thiazolocarbocyanines were obtained when alkyl iodides of the specified thiazole bases were condensed in the presence of alkyl orthoformate and pyridine. As herein described, alkyl ortho-esters of a mono-carboxylic acid having more than one carbon atom yield 7-substituted thiazolocarbocyanines. These are related to the neothiazolocarbocyanines in that both dyes have a univalent group attached to the carbon atom in the 7-position.

39 It is, therefore, among the objects of the present invention to provide a process for the preparation of the thiazolocarbocyanines. A further object is to provide a process for the preparation of the 7-substituted thiazolocarbocyanines. Other objects will appear upon a further perusal of this specification.

The thiazole bases with a reactive methyl group in the 2-position may be given the general formula—



where A and B represent univalent atoms or groups such as hydrogen, aliphatic or aromatic groupings. The numbering is that in common usage for bases of this type, being that used, for instance in Richter's Lexikon der Kohlenstoff Verbindungen.

The base 2-methylthiazole, or a substituted 2-methylthiazole, e. g. 2-methyl-4-phenylthiazole, may be converted into an alkylquaternary salt by heating it with, for instance, a dialkyl sulfate or

an alkyl p-tolene sulfonate or an alkyl iodide. When the alkyl halides are used, quaternary alkyl iodides are produced which on treatment with ethylorthoformate and pyridine under appropriate conditions yield thiazolocarbocyanines.

The general reaction of alkyl quaternary salts of 2-methylthiazoles with alkyl ortho esters of the monocarboxylic acids may be written as follows—



In the above equation A and B have the significance given to them above, R stands for alkyl and X is a suitable acidic radical. The acidic radical X may be changed at will by using the various methods of double decomposition. If the reaction has been carried out using the p-toluenesulfonate radical, for example, the dye may be readily precipitated as the less soluble iodide by adding an aqueous solution of potassium iodide. R<sup>1</sup> and R<sup>2</sup> are likewise alkyl groups and may be similar or dissimilar. There is a method for the preparation of orthoesters of monocarboxylic acids (see my U. S. Patents Nos. 1,846,301, 2, 3 and 4) which may be used so as to give ortho esters in which R<sup>1</sup> and R<sup>2</sup> are similar or dissimilar but, as may be seen from the equation, these alkyl groups are removed as molecules of alcohol and do not enter the dye molecule. D is a suitable univalent atom or group, such as hydrogen, alkyl or aryl. If D be hydrogen then the ester employed is derived from orthoformic acid and X is best chosen as iodide for the main product of the reaction to be normal thiazolocarbocyanine 30 35 40 45 50 of the type:



as has already been explained, since choice of, for example, p-toluenesulfonate for **X** results in a preponderance of the special type of 7-substi-

tuted thiazolocarbocyanines known as neothiazolocarbocyanines. In most cases however, some normal thiazolocarbocyanine is produced even when  $X$  is p-toluenesulfonate or alkylsulfate, but if the normal compound is desired it is recommended that iodide be chosen for  $X$  and this results in the product in general being almost pure normal compound.

If  $D$  represent a univalent group such as methyl or ethyl ( $CH_3$ — or  $C_2H_5$ —) then it is immaterial whether  $X$  represents halide, p-toluenesulfonate, alkylsulfate or the like, as far as the type of compound is concerned. In all cases the 7-substituted dye is produced. The yield of product, however, may vary with the acidic radical employed, and in general an aryl sulfonic radical is preferred for the condensations.

These new dyes are useful as sensitizers for photographic emulsions, such as gelatino-silver-halide emulsions, for the green portion of the spectrum.

The 2-methylselenazoles may be regarded as thiazoles in which the sulfur atom in the molecule has been replaced by a selenium atom. These new bases are described in my co-pending application with Frank L. White No. 619,959 filed of even date. Selenazolocarbocyanine dyes derived from the 2-methylselenazoles may be prepared in a manner similar to that herein described for the thiazolocarbocyanines.

In general it is desirable to employ an excess of the ortho ester over the amount (one molecular proportion of ester to two molecular proportions of quaternary salt) shown in the equation. This results in an increase in yield. The ortho ester and the quaternary salts are conveniently condensed together by refluxing them together in anhydrous pyridine, usually for an hour or longer. After the reaction is finished the dye may be precipitated as a tar by the addition of ether, the ethereal layer decanted and the tar dissolved in a little hot alcohol (methyl or ethyl) and precipitated as, for instance, the iodide by an excess of aqueous potassium iodide, or in some cases the dye may be precipitated from the pyridine reaction mixture by the addition of water, and in still other cases the dye separates from the reaction mixture in the crystalline state. These methods are all simple procedures and are well known in the art.

#### EXAMPLE I

##### *3,3',4,4'-tetramethylthiazolocarbocyanine iodide*

2.6 parts of 2,4-dimethylthiazole methiodide were refluxed for 5 hours in 30 parts of pyridine with 3 parts of ethyl orthoformate. After allowing the reaction mixture to cool the dye was filtered off and impurities removed by washing with water. The dye was recrystallized from methyl alcohol and was obtained in dark blue needles which gave a crimson solution in the solvent.

#### EXAMPLE II

##### *4,4' - dimethyl-3,3' - diethylthiazolocarbocyanine iodide*

2,4-dimethylthiazole ethiodide was made by refluxing the base with ethyl iodide for several days and washing the solid product with acetone to remove starting materials.

2.7 parts of this ethiodide were refluxed for 5 hours with 30 parts of pyridine and 3 parts of ethyl orthoformate. The dye was precipitated

by diluting the reaction mixture with an equal volume of water and allowing to cool. The product was recrystallized from methyl alcohol in which it gave a crimson solution and was obtained in dark needles with a greenish reflex.

It has been described in my co-pending application No. 548,025 Example V, that this dye may also be obtained together with the corresponding neothiazolocarbocyanine. The "almost pure normal thiazolocarbocyanine" described in that example may be given a further crystallization to render it completely pure.

#### EXAMPLE III

##### *4,4' - diphenyl-3,3' - dimethylthiazolocarbocyanine iodide*

4-phenyl-2-methylthiazole methiodide was prepared by refluxing equal weights of 4-phenyl-2-methylthiazole and of methyl iodide for two days. The solid alkyl quaternary salt was removed, ground finely under acetone, filtered off and washed with acetone and dried.

2 parts of the methiodide obtained above were refluxed with 25 parts of pyridine and 2 parts of ethyl orthoformate for 1½ hours. The reaction mixture was diluted with 60 parts of warm water and allowed to cool overnight. The dye separated out and was filtered off, washed with water and then purified by recrystallization from methyl alcohol. The dye was obtained as small dark compact crystals with a greenish lustre and gave a crimson solution in methyl alcohol. No bluish neothiazolocarbocyanine was encountered at all in this preparation.

#### EXAMPLE IV

##### *4,4' - diphenyl-3,3' - diethylthiazolocarbocyanine iodide*

4-phenyl-2-methylthiazole ethiodide was prepared by heating 4-phenyl-2-methylthiazole with ethyl iodide under reflux for 50 hours. The solid ethiodide was removed, pulverized and washed free from starting materials with acetone. 3.3 parts of the salt were heated under reflux with 30 parts of anhydrous pyridine and 3 parts of ethyl orthoformate for 1½ hours. The reaction mixture was then diluted with an equal volume of water and allowed to cool. Bronze crystals of the dye separated out which were purified by recrystallization from a small quantity of methyl alcohol. The dye formed small greenish crystals and gave a crimson solution in the solvent.

#### EXAMPLE V

##### *4,4' - dimethyl-3,3',7-triethylthiazolocarbocyanine iodide*

2.25 parts of 2,4-dimethylthiazole were converted into the etho-p-toluenesulfonate of the base by heating it with 4 parts of ethyl-p-toluenesulfonate at 130-140° C. for six hours. The crude quaternary salt (a viscous melt) was then refluxed without further purification with 20 parts of pyridine and 7 parts of ethyl ortho-propionate for 2½ hours. After allowing the reaction mixture to cool, the dye was precipitated by the addition of ether, the ethereal layer decanted off and the tar dissolved in a little warm methyl alcohol and precipitated as the iodide by adding thereto a solution of 10 parts potassium iodide dissolved in 100 parts of water. After allowing the whole to stand aside for several days the dye was removed by filtration and purified by

washing followed by recrystallization from methyl alcohol in which it gave a beautiful crimson solution. The dye, after filtration and air-drying, was obtained as dark needles with a green reflex.

EXAMPLE VI

4,4'-diphenyl-3,3',7-trimethylthiazolocarbocyanine iodide

- 10 3.5 parts of 4-phenyl-2-methyl thiazole were converted into the metho-p-toluenesulfonate of the base by heating with 3.7 parts of methyl-p-toluenesulfonate at 100° C. overnight. The crude 4-phenyl-2-methylthiazole metho-p-toluenesulfonate was then refluxed for 90 minutes with 10 parts of pyridine and 4.8 parts of methyl ortho-acetate. The dye was then precipitated as the sparingly soluble iodide by double decomposition with a solution of 5 parts of potassium iodide in 20 50 parts of hot water. The dye separated as a tarry residue, and after the aqueous liquor had been removed, this residue was washed. The purplish black powder was purified by recrystallization from methyl alcohol and the dye was thus obtained as small greenish crystals with a bright lustre. The solution of the dye in methyl alcohol was a crimson color.

EXAMPLE VII

30 4,4'-diphenyl-3,3'-dimethyl-7-ethylthiazolocarbocyanine iodide

- 35 3.5 parts of 4-phenyl-2-methylthiazole were condensed with 3.7 parts of methyl-p-toluenesulfonate as described in Example VI. The quaternary salt was refluxed without further purification with 5.4 parts of methyl ortho-propionate and 10 parts of pyridine for 90 minutes. The dye was precipitated as the iodide exactly as described for the dye in Example VI and was purified and recrystallized in the same manner also. The dye gave a crimson solution in methyl alcohol and crystallized in small green crystals with a green luster.

- 45 From the foregoing it becomes apparent that thiazolocarbocyanines may be prepared by condensing two molecular proportions of a 2-methylthiazole alkyl quaternary salt with one molecular proportion of an ortho ester of a monocarboxylic acid. The thiazole may have either hydrogen or a suitable univalent group in one or both of the 4, 5 positions. If an ortho ester of formic acid is employed, an unsubstituted thiazolocarbocyanine will be obtained. If an ortho ester of a monocarboxylic acid other than formic acid is employed, a 7-substituted thiazolocarbocyanine is obtained. These ortho esters are described in my Patents Numbers, 1,846,301, 2, 3 and 4, and need not be repeated here.

- 55 Other variations and equivalents will doubtless occur to those skilled in this art, it being understood that the foregoing is stated only to illustrate to those skilled in the art how thiazole alkyl quaternary salts may be condensed with an ortho ester of a monocarboxylic acid to form a thiazolocarbocyanine.

What I claim as my invention and desire to secure by Letters Patent of the United States is—

- 60 1. A process for the preparation of thiazolocarbocyanines which comprises condensing, under the influence of heat, two molecular proportions of a thiazole alkyl quaternary salt with one molecular proportion of an ortho-ester of an aliphatic monocarboxylic acid in the presence of an organic base which is a solvent for the reactants

and which acts to bind acid eliminated from the quaternary salt as a result of the condensation.

65 2. A process for the preparation of thiazolocarbocyanines which comprises condensing one molecular proportion of an ortho-ester of an aliphatic monocarboxylic acid, under the influence of heat, with two molecular proportions of an alkyl quaternary salt represented by the following structure:



70 in which A and B represent hydrogen, an aliphatic group or an aromatic radical of the benzene series, R represents alkyl and X represents an acid radical.

75 3. A process for the preparation of thiazolocarbocyanines which comprises condensing, under the influence of heat, two molecular proportions of a thiazole alkyl quaternary salt with one molecular proportion of an ortho-ester of an aliphatic monocarboxylic acid in the presence of an organic base which is a solvent for the reactants and which acts to bind acid eliminated from the quaternary salt as a result of the condensation.

80 4. A process for the preparation of thiazolocarbocyanines which comprises condensing, under the influence of heat, two molecular proportions of a thiazole alkyl quaternary salt with one molecular proportion of an alkyl ortho-formate in the presence of an organic base which is a solvent for the reactants and which acts to bind acid eliminated from the quaternary salt as a result of the condensation.

85 5. A process for the preparation of thiazolocarbocyanines which comprises condensing, under the influence of heat, two molecular proportions of a thiazole alkyl quaternary salt with one molecular proportion of an alkyl ortho-acetate in the presence of an organic base which is a solvent for the reactants and which acts to bind acid eliminated from the quaternary salt as a result of the condensation.

90 6. A process for the preparation of thiazolocarbocyanines which comprises condensing, under the influence of heat, two molecular proportions of a thiazole alkyl quaternary salt with one molecular proportion of an ortho-ester of a monocarboxylic acid in the presence of pyridine.

95 7. A process for the preparation of thiazolocarbocyanines which comprises condensing, under the influence of heat, two molecular proportions of a thiazole alkyl quaternary salt with one molecular proportion of an alkyl ortho-formate, in the presence of pyridine.

100 8. A process for the preparation of thiazolocarbocyanines which comprises condensing, under the influence of heat, two molecular proportions of a thiazole alkyl quaternary salt with one molecular proportion of an alkyl ortho-acetate in the presence of pyridine.

9. A carbocyanine dye of the following structure



105 in which A and B represent hydrogen, an aliphatic group or an aromatic radical of the benzene series, R represents alkyl and X represents an acid radical.

phatic group or an aromatic radical of the benzene series, R equals alkyl, X equals an acid radical and D equals an alkyl group or an aryl group of the benzene series.

- 5 10. A carbocyanine dye of the following structure



in which A and B represent hydrogen, an aliphatic group or an aromatic radical of the benzene series, R equals alkyl, X equals an acid radical and D equals an alkyl group.

11. A carbocyanine dye of the following structure



25 in which A and B represent hydrogen, an aliphatic group or an aromatic radical of the benzene series, R equals alkyl, X equals an acid radical and D equals an alkyl group or an aryl group of the benzene series.

phatic group or an aromatic radical of the benzene series, R equals alkyl, X equals an acid radical and D equals a methyl group.

12. A carbocyanine dye of the following structure



in which A and B represent hydrogen, an aliphatic group or an aromatic radical of the benzene series, R equals alkyl, X equals an acid radical and D equals an ethyl group.

13. A 3,3'-dialkyl-7-alkyl-thiazolocarbocyanine salt.

14. A 3,3'-dialkyl-7-methyl-thiazolocarbocyanine salt.

15. A 4,4'-dialkyl-3,3'-dialkyl-7-alkyl-thiazolo- 20 carbocyanine salt.

16. A 4,4'-diaryl-3,3'-dialkyl-7-alkyl-thiazolo- carbocyanine salt the aryl groups being of the benzene series.

LESLIE G. S. BROOKER. 25